

Dec. 13, 1932.

W. KRAUSS

1,891,097

COPPER IODIDE RECTIFIER

Filed Sept. 8, 1930

Fig. 1



Fig. 2



Inventor:  
Walther Krauss,  
by *Charles E. Tulla*  
His Attorney.

## UNITED STATES PATENT OFFICE

WALTHER KRAUSS, OF BERLIN-ZEHLENDORF, GERMANY, ASSIGNOR TO GENERAL ELECTRIC COMPANY, A CORPORATION OF NEW YORK

## COPPER IODIDE RECTIFIER

Application filed September 8, 1930, Serial No. 480,404, and in Germany October 3, 1929.

My invention relates to alternating current rectifiers of the solid electrode or dry plate type, particularly to rectifiers of this type comprising copper iodide elements, and 5 its object is the provision of an improved copper iodide rectifier and of an improved method of preparing the elements therefor.

In the use of dry rectifiers in which the discs are built up of copper iodide in contact 10 with electrodes of various materials, it has been observed that the rectifying effect weakens after a comparatively short period of operation. It is believed that this disadvantageous action of the copper iodide rectifiers 15 previously known is due to a polarization effect, since experiments in which the rectifiers were subjected to the action of direct current before being used for the rectification of alternating current have shown that in the use 20 of such rectifiers the ratio of the alternating current supplied to the rectifier to the direct current output thereof is dependent on the direction, amount and duration of the direct current passed through the rectifier in this 25 preliminary treatment, and that such preliminary treatment with direct current exerts, in general, an unfavorable influence on the ratio of input to output of the rectifier.

In accordance with my invention, the injurious action of the above-noted polarization 30 effect is substantially eliminated by the addition to the copper iodide of oxidizing means, preferably iodine. I have found that by the addition of a suitable amount of iodine to 35 the copper iodide, the ratio of alternating current input to the direct current output of the copper iodide rectifier becomes substantially independent of the preliminary treatment with direct current, and at the same time 40 much longer operating life of the rectifier is attained. If curves were drawn which represented the ratio of alternating current input 45 to direct current output in dependence on the preliminary treatment with direct current, for example, to a given duration of the

time of preliminary treatment  $t$ , they would show an average slope,

$$\frac{\Delta \frac{(\text{a. c. input})}{(\text{d. c. output})}}{\Delta t} \quad 50$$

of 1.34 if iodine were not added to the copper iodide. But if iodine were added, the average slope of the curves would be only 55 0.0016, the slope in the latter case thus being of an entirely different order of magnitude.

Favorable results similar to those described above are attained when other oxidizing means instead of iodine are added to the 60 copper iodide, such as persalts or peroxides.

My invention will be better understood 65 from the following description when considered in connection with the accompanying drawing and its scope will be pointed out in the appended claims.

Referring to the drawing, Figs. 1 and 2 are respectively a plan view and cross-section of a rectifier disc embodying my invention.

In the figures a single rectifier disc 1 is 70 shown comprising a comparatively massive plate of copper iodide 2 between a lead plate 3 and a layer of copper 4. The plate 3 may be of thin lead foil on which has been formed a layer of lead sulphate 5; the layer 4 preferably consists of finely powdered copper. In forming the complete disc 1, lead plate 3 is placed at the bottom of a die in a press and iodide mixture is poured on the lead. After the iodide has been pressed lightly to 75 produce a smooth surface the copper powder is distributed uniformly over the surface. The layers are then pressed together strongly and a hard, dense disc is thus obtained. As hereinbefore explained, in accordance with 80 the present invention means are provided to avoid the polarization difficulties heretofore encountered in the use of copper iodide rectifiers. To this end, the material forming 85 the layer 2 is not copper iodide alone but con- 90

sists of pure copper iodide to which has been added a suitable oxidizing agent, preferably free iodine, to the extent, for example, of 0.3%. The lead sulphate 5 on the surface of plate 3 facilitates the formation of a thin coating of lead iodide 6 on the lead plate by the action of the free iodine in the copper iodide after the operation of pressing up of the disc, and this thin coating of lead iodide is the seat of the rectification of alternating current when the disc is incorporated in a rectifier circuit.

10 What I claim as new and desire to secure by Letters Patent of the United States is:

15 1. A rectifier comprising a lead electrode having a lead sulphate surface formed thereon, and an element in contact with said surface comprising a mixture of copper iodide and free iodine.

20 2. The combination in a rectifier of a lead electrode, a layer of lead sulphate on the surface of said electrode, an element comprising copper iodide and free iodine mixed therewith, and a coating of lead iodide formed

25 by the action of said iodine on said lead sulphate between said lead electrode and said element.

30 In witness whereof, I have hereunto set my hand this 19th day of August, 1930.

WALTHER KRAUSS.

35

40

45

50

55

60

65